

March 18, 1941.

H. N. GILBERT

2,234,967

PRODUCTION OF ALKALI METALS

Original Filed March 11, 1936 2 Sheets-Sheet 1



March 18, 1941.

H. N. GILBERT

2,234,967

PRODUCTION OF ALKALI METALS

Original Filed March 11, 1936

2 Sheets-Sheet 2



Fig. 3



Fig. 2

INVENTOR.  
HARVEY N. GILBERT  
BY *Harold J. Budrow*  
ATTORNEY

## UNITED STATES PATENT OFFICE

2,234,967

## PRODUCTION OF ALKALI METALS

Harvey N. Gilbert, Niagara Falls, N. Y., assignor  
to E. I. du Pont de Nemours & Company, Wil-  
mington, Del., a corporation of Delaware

Application March 11, 1936, Serial No. 68,274  
Renewed May 17, 1940

3 Claims. (Cl. 204—21)

This invention relates to the electrolysis of alkali metal compounds to produce alkali metals and other valuable products and more particularly to electrolysis processes which utilize liquid metal electrodes.

Various methods and apparatus for electrolysis of alkali metal compounds, either in the fused state or in aqueous solutions, with the use of circulating liquid metal electrodes are well known.

10 An example of this is the well-known Castner cell used for the production of caustic soda, wherein mercury serves as the cathode for the electrolysis of aqueous sodium chloride solution. In processes of this nature, the alkali metal released at the liquid metal cathode alloys therewith and the resulting liquid alloy then is circulated to react chemically with water or other substances to produce caustic soda or other sodium compounds. In such processes proposed heretofore, the liquid metal serving as electrode has been circulated 15 through the cell in a relatively shallow layer of wide dimensions, so as to expose a relatively large electrode surface to the electrolyte. These methods require relatively large amounts of the liquid metal, which is usually molten lead or mercury, and considerable power is expended in the circulation thereof. An important factor in the economies of such liquid metal electrode cells is the large amount of floor space required, as compared with other types of electrolytic cells which may have all electrodes vertical.

15 A number of methods have been proposed for producing metallic sodium by the use of a two-cell system employing a liquid metal electrode whereby a fused salt is first electrolyzed with a liquid metal cathode to form the sodium alloy and this liquid sodium alloy then is used as anode in a cell employing a fused sodium compound as electrolyte, e. g. caustic soda, whereby metallic sodium is released at the cathode. This method of producing sodium has not enjoyed any substantial commercial use and so far as I am aware is not commercially used at the present time. A significant disadvantage of this two-cell system 20 of producing sodium has been the excessively high temperatures used. These high temperatures, e. g. 350° C. or higher, make it difficult to employ mercury as liquid electrode because of the relatively high vapor pressure of mercury at these 25 temperatures. A further disadvantage of the high temperatures is that the working life of the equipment is seriously shortened because of the tendency of rapid corrosion at high temperatures and also because of energy loss in the 30 form of radiated heat.

An object of this invention is to provide an improved method and means for electrolysis of alkali metal compounds utilizing a liquid metal electrode by which higher electrical efficiencies may be obtained, a greater amount of liquid electrode surface is exposed to the electrolyte for a given amount of floor space and a smaller amount of liquid metal serving as electrode is required in a cell of given capacity than has been heretofore possible. A further object is to provide an improved method for producing alkali metal by a two-cell method utilizing liquid metal electrodes, with higher overall current efficiency, utilization of less liquid metal and exposure of greater liquid metal electrode surfaces to the electrolytes for given floor space than has heretofore been possible. A still further object is to provide an efficient double-cell process for producing alkali metal wherein an aqueous solution is electrolyzed with a liquid cathode to produce liquid 10 alkali metal alloy and this liquid alloy is used as anode in a fused salt electrolysis to recover alkali metal from said alloy. Another object is to provide improved method and apparatus for reacting alkali metal amalgam with liquid or gaseous reagents to produce valuable alkali metal products, e. g., reaction with water to produce the hydroxides. Other objects will be apparent from the following description of my invention.

In accordance with the present invention, I 30 attain the objects stated above essentially by providing a moving or movable electrode structure which is coated with an adherent film of the liquid metal utilized as electrode. I may also provide means for contacting this electrode structure with a body of the liquid electrode to replenish the liquid metal film thereon. In the preferred embodiment of my invention I provide a moving metal surface which is adapted continuously or intermittently to be passed through or 35 dipped into a reservoir of the liquid metal serving as electrode and after being thus contacted with the liquid metal to pick up an adherent film thereon, to be contacted with the electrolyte, whereupon the film of liquid metal may serve as 40 electrode. In this manner, I utilize a thin film of the liquid metal or alloy as effective electrode, in place of the relatively large bodies or pools of liquid which have been employed heretofore. The moving surface of solid conductive material, to 45 which the liquid metal film adheres, serves to continuously replenish the film in contact with the electrolyte.

In the appended drawings a preferred embodiment of the apparatus of my invention is illus- 50 55

trated. Fig. 1 is a vertical sectional view of a two-cell system embodying my invention. Figs. 2 and 3 are sections at right angles to the section of Fig. 1, of parts of the apparatus illustrated in Fig. 1.

The drawings illustrate a two-cell system suitable for electrolyzing sodium chloride to produce chlorine and metallic sodium in accordance with my invention. This apparatus comprises a "cold cell" in which an aqueous salt solution may be electrolyzed and a "hot cell" in which a molten sodium compound or a fused mixture of sodium compounds may be electrolyzed. The "cold cell" is shown in section at the left hand side of Fig. 1 and by Fig. 2, which is a section in plane AA of Fig. 1. The shell or container 1, which may be constructed of concrete or other suitable material, has three semicircular wells 2 cast in the bottom thereof. Three vertical wheels 3 are mounted on a rotatable shaft 4 supported by bearings 7 in such manner that the lower part of the wheels 3 depend into the wells 2. The upper part of the cell is covered with a dome shaped gas collector 8 which is made of material resistant to chlorine, preferably ceramic material. Through openings in the top of dome 8 are suspended four vertical anodes 9, preferably made of graphite. The anodes 9 are connected to an electrical lead or bus bar 10. Outlet pipe 11, made of chlorine-resistant material is provided in the top of dome 8 to conduct evolved gas from the interior of the cell. The upper portion of the cell is provided with inlet pipe 12, for introducing an aqueous electrolyte into the cell and outlet pipe 13 for removing aqueous electrolyte from the cell. By means of suitable electrolyte reservoir and pump arrangement not shown, the aqueous electrolyte may be circulated through the cell by way of pipe 12 and 13. The shaft 4, upon which is mounted the rotating wheels 3, is caused to rotate by means of gears 5 and shaft 6 which is connected to a suitable source of power not shown.

In operating this apparatus in accordance with one embodiment of my invention, the "cold cell" illustrated in the drawings is filled with mercury or other liquid metal or alloy up to a point below the lower ends of the anodes 9. The liquid metal electrode must have a melting point below the boiling point of the aqueous electrolyte used, unless pressure is applied; mercury is preferred for the metal electrode. The liquid metal may enter the cell by means of pipe 17 and may be removed therefrom by way of pipes 14 which are connected to the bottom of the wells 2. The upper portion of the cell above the liquid metal level is filled with an aqueous alkali metal salt solution, e. g. a solution of sodium chloride, preferably to a point somewhat above the tops of the rotating wheels 3. In the preferred operation of this cell, brine is continuously circulated through the upper portion of the cell and simultaneously the liquid metal which may serve as cathode is continuously circulated through the lower portion of the cell by way of pipes 14 and pipe 17. Preferably the liquid metal enters at a point near the upper surface of the liquid metal through pipe 17 and is withdrawn from the bottom of the cell through pipes 14. This circulation, however, may occur in reverse direction from that stated if desired.

In the specific modification illustrated by the drawing in Fig. 1 the "cold cell" is operated in conjunction with a "hot cell" of similar construction and the two cells are connected by a

suitable arrangement of conduits for circulating the liquid metal electrode through each cell and from one cell to the other. The preferred modification includes a heat exchanger 18, whereby the liquid metal leaving the "hot cell" is cooled before it enters the "cold cell" and the liquid metal leaving the "cold cell" is heated before it enters the "hot cell." In addition to the use of the heat exchanger, it is sometimes advisable to provide an additional cooling means for cooling the metal leaving the heat exchanger before it enters the "cold cell." Such cooling means (not shown) may be of any conventional design. Referring to Figs. 1 and 3, the "hot cell" suitable for the production of alkali metal by electrolysis of the fused alkali metal compound in conjunction with an alkali metal alloy as liquid metal anode will be described. The "hot cell" is shown in section at the right hand side of Fig. 1; Fig. 3 is a cross section of the "hot cell" on the plane BB shown in Fig. 1. The "hot cell" construction includes a shell or container the lower part of which 23 is of relatively heavy construction, e. g. cast iron or cast steel, while the upper part 24 is of some lighter construction, e. g. steel plate. The lower half 23 of the cell is provided with three depressions or wells 25 the cross sections of which, as shown in Fig. 3, are semicircular in shape. A shaft 27 extends transversely of the cell mounted on bearings 21, this shaft being provided with gears 28 and counter-shaft 29, the latter being connected to a suitable source of power not shown for rotating shaft 27. Three wheels 26 are attached to the shaft 27 so as to rotate therewith, the lower portions of wheels 26 depending into the wells 25. In upper portion of the cell are four metallic cathodes 30, preferably made of steel, which are suspended on the horizontal metallic member 31. Horizontal member 31 in turn is suspended from bus bar 32 which extends through the dome 33 to a point outside the cell. Collecting dome 33, preferably constructed of cast steel, is mounted above the cathodes 30 and serves to collect molten metal liberated at the cathodes and rising therefrom. Pipe 36 connected to the top of dome 33 is provided to carry off the collected molten cathodic product into receiver 37 to which it is connected. Receiver 37 is fitted with valves 38 at its lower end, whereby the collected molten metal may be removed from time to time. Pipes 39 connected with the bottoms of the wells 25, together with pipe 22, are provided for circulating molten metal anode through the cell. In the upper portion of the cell is suspended a vertical shield 34, extending completely around all sides of the cell, spaced a short distance away from the side walls 4. The shield 34, extends downward to a point just above but out of contact with the level of the liquid metal anode in the cell and is supported at its upper end by means of electrical insulation 35 which in turn is supported by the outstanding flange of the side wall 24. The entire cell preferably is covered with a layer of heat insulating material 40. The "hot cell" may be supported by I-beams 42, as shown in Fig. 3. I prefer to provide the cell with a cover 44 to prevent access of air to the electrolyte.

In the operation of the "hot cell" the lower portion is filled with the circulating liquid metal anode preferably to a point slightly above the axis of the rotating wheels, and space above the liquid metal anode is filled with a molten alkali metal compound or a fused mixture of alkali metal compounds to serve as electrolyte. A

liquid metal alloy of an alkali metal, e. g. sodium amalgam, is circulated through the lower part of the "hot cell" to serve as anode. On passage of the electrical current, alkali metal is dissolved from the anode and liberated at the cathode. The cathodic product, which is in the liquid state rises in the collector dome 33 and thence flows through pipe 36 to receiver 31. The temperature of the molten electrolyte may be regulated 10 by adjusting the flow of electrical current. If desired, the temperature may additionally be regulated by the use of suitable heating and/or cooling means in contact with the electrolyte.

To provide for circulating the liquid metal serving as electrodes in the hot and cold cells, pipe 15 conducts the liquid metal from pipe 14 in the bottom of the "cold cell" to pump 16 which elevates the metal and forces it through the heat exchanger 18. From the heat exchanger 18, the liquid metal flows through pipe 21 and enters the bottom of the "hot cell" by way of pipes 39. The liquid metal leaves the "hot cell" by way of pipe 22, near the surface of the liquid metal in the "hot cell" and thence flows by gravity 25 through the heat exchanger 18 and thence through pipe 17 into the "cold cell." Heat exchanger 18, which is illustrated diagrammatically in Fig. 1, may be of conventional design. Preferably, it is covered with a layer of heat insulating material 19. Likewise, pipe 21, leading from the heat exchanger to the "hot cell" may be covered with heat insulation 43.

The purpose of the shield 34 in the "hot cell" is to prevent the walls 24 from acting as anode, since walls 24 are in electrical connection with the liquid metal anode in the lower part of the cell. It was found that heat resistant insulating materials which would be suitable in the construction for maintaining the liquid metal anode out of electrical contact with that portion of the cell which is in contact with the molten electrolyte, tended slowly to dissolve in the electrolyte and thus to contaminate it. This was found to be the case, for example, when a slab of marble was used as insulator in contact with the electrolyte, the marble slowly dissolving to introduce calcium into the electrolyte which increased the viscosity and melting point of the electrolyte and tended to contaminate the cathodic product with calcium. By means of shield 34, which is maintained out of electrical contact with the side walls 24 by means of insulator 35, it was found that the anodic effect of wall 24 was substantially completely eliminated.

In the operation of the "hot cell" the concentration of alkali metal in the liquid metal anode introduced into the cell may vary within wide limits. I have found that when using mercury as the liquid metal, there is no advantage in increasing the alkali metal content of the anode above about 0.2% by weight; at higher concentrations the viscosity of the amalgam may become excessively high. In the production of sodium, I prefer to maintain the sodium concentration of the liquid metal entering the "hot cell" at 0.03 to 1.0% by weight.

In general the operation of my improved electrolytic cell as above illustrated is similar, regardless of whether it is used as "cold cell" whereby the liquid metal is used as cathode or as a "hot cell" wherein a liquid metal alloy of an alkali metal is used as anode. The principle of the operation is to rotate the wheels 3 or 26, 70 whereby the surfaces of the wheels continuously

pass first through the molten metal and then through the electrolyte. For example in the operation of the "cold cell" the aqueous electrolyte may be a solution of sodium chloride and the liquid metal cathode may be chiefly mercury or mercury alloy. As the wheel rotates through the mercury cathode a thin film of mercury adheres to the surface of the wheel and this thin film of mercury is brought into contact with the aqueous electrolyte by the rotation of the wheel. In this manner a relatively large surface of mercury is brought into contact with the electrolyte and a rapid electrolysis ensues, liberating metallic sodium at the surface of the cathode film. The sodium alloys with the cathode film and as the wheel rotates, the resulting amalgam then comes into contact with the mercury or weak amalgam which is circulated through the bottom portion of the cell. It should be stated at this point that when the surface of the wheels 3 is made of a metal such as iron or steel with which mercury does not readily alloy or the surface of which mercury does not readily "wet," pure mercury will not readily adhere to the surface of the wheel. I have discovered that if the mercury initially contains a small amount of alkali metal, the mercury will readily adhere to an iron or steel surface which is reasonably clean to form a continuous film thereon. For example, I have found that a sodium amalgam containing not less than about 0.01% by weight of sodium will wet a clean plain carbon steel surface, while amalgam less rich in sodium will not. Metals other than ordinary steel which are suitable for the surface of the wheel may require different amounts of sodium in the amalgam to wet the metallic surface. Likewise the required amount of alkali metal in the amalgam to wet a given metal surface will vary for different alkali metals. The following tabulation shows the approximate minimum concentrations of sodium and potassium in the amalgam required to readily wet different metallic surfaces:

| Metal surface                      | Approximate minimum concentration of alkali metal in amalgam |                   | 45 |
|------------------------------------|--------------------------------------------------------------|-------------------|----|
|                                    | Sodium                                                       | Potassium         |    |
| Stainless chrome steel.....        | Percent by weight                                            | Percent by weight |    |
| Monel metal.....                   | 0.05                                                         | 0.15              |    |
| Carbon steel (S. A. E. 10-10)..... | 0.01                                                         | 0.10              |    |
| Nickel.....                        | 0.01                                                         | 0.05              | 50 |
|                                    |                                                              | 0.02              | 55 |

In practicing my invention to electrolyze aqueous solutions of alkali metal salts, I prefer to coat the rotatable wheel or equivalent means utilized with an adherent layer of the amalgam prior to starting the electrolysis. This is done to prevent chemical reaction between the metal of which the wheel is made and the electrolyte or electrolysis products. For example if the wheel is made of iron or steel in the electrolysis of sodium chloride, when electrolysis is started any iron in contact with the electrolyte may react to form hydrogen. The hydrogen, mixing with the chlorine may form an explosive mixture. Hence it is desirable to keep the wheel completely covered with an adherent layer of amalgam at all times. To coat the wheel with amalgam prior to electrolysis, I may dissolve sufficient alkali metal in the mercury to cause wetting, (as illustrated by the above tabulation) and revolve the 75

wheel therein until it is covered with the amalgam. The electrolysis then may be started. By this means, the entire working surface of the wheel will have a uniform, adherent coating of amalgam which prevents contact of the base metal with the electrolyte during the electrolysis.

If the cell is constructed of metal which readily alloys with mercury, e. g. copper or brass, it will not be necessary to have alkali metal initially present in the liquid metal electrode. However, it is preferable to use iron, an iron alloy (e. g. steels), nickel, or a nickel alloy (e. g. Monel metal) for the wheel construction, since such metals do not readily alloy with mercury and hence resist corrosion by the mercury. Chromium-iron alloys such as "stainless steel" are suitable for this purpose.

In the operation of a "hot cell" in the utilization of my invention the general considerations above recited in regard to the operation of the "cold cell" will apply. For example by circulating an alloy of sodium and mercury through the lower portion of the "hot cell" to serve as anode and utilizing a molten sodium compound, e. g. 20 NaOH, as electrolyte, metallic sodium will be electrically dissolved from the liquid metal anode and liberated at the cathode from whence it rises by reason of its low specific gravity into the upper portion of the collecting dome 33 and hence through a pipe 36 into the receiver 37. In 25 the operation of a "hot cell" of this character it is desirable to maintain as low a temperature as possible because of the tendency for mercury to vaporize at elevated temperatures, because of loss 30 of energy by way of radiated heat at excessively high temperatures and because of damage caused to cell parts by warping and corrosion which is liable to occur if excessive temperatures are used.

The molten electrolyte in the "hot cell" preferably should have a melting point not higher than 40 about 250 to 300° C., if the liquid metal electrode flowing between the two cells is mercury or alkali metal amalgam, since the vapor pressure of mercury becomes excessively high at temperatures 45 much above 300° C. I prefer to use an electrolyte of sufficiently low melting point so that the temperature of the fused electrolyte can be maintained at not higher than 240 to 300° C. Heretofore, it has not been practicable to utilize mercury as exchange electrode in a two cell system with fused electrolyte because of the relatively high melting point of the electrolytes which has made necessary the use of temperatures of about 50 350° C. and higher. The operator therefore 55 was forced to use molten lead as electrode and this prevented the use of a "cold cell" in conjunction with the "hot cell."

As disclosed and claimed in my co-pending application filed of even date herewith, I have 60 discovered that various mixtures of alkali metal hydroxide and alkali metal halides may be prepared having melting points lower than about 300° C. and as low as around 200° C. For example, in the production of sodium by the double-cell system described above, using mercury as exchange electrode, I may use a mixture of sodium hydroxide and sodium iodide which has a melting point not higher than 300° C. Preferably, I use the eutectic mixture of these compounds 65 containing about 55% by weight of sodium hydroxide and 45% sodium iodide which melts at about 225° C. or an approximation thereof. With this eutectic mixture, the cell advantageously may be operated at a temperature of 240 to 250° 70 75 C. at which temperature the vapor pressure of

mercury is only about one-tenth of one atmosphere. Alternatively, I may use the eutectic mixture of sodium hydroxide and sodium bromide, which melts at about 260° C. Other similar mixtures may be used for the production of other alkali metals or for the production of mixtures of alkali metals, in accordance with my invention. For example, the following eutectic mixtures may be used.

| Eutectic mixture                | Melting point | 10 |
|---------------------------------|---------------|----|
| NaOH (79 molar percent) + NaBr  | 260           |    |
| KOH (72 molar percent) + KI     | 250           | 15 |
| KOH (65 molar percent) + KBr    | 300           |    |
| LiOH (48.5 molar percent) + LiI | 180           |    |
| LiOH (45 molar percent) + LiBr  | 275           |    |
| LiOH (63 molar percent) + LiCl  | 290           |    |

I have found that such fused mixtures of alkali metal hydroxides and alkali metal halides may be electrolyzed with an alkali metal alloy anode over long periods of time with substantially no decomposition or change in composition to electrolytically dissolve alkali metal from the anode and liberate it at the cathode.

The speed of rotation of the electrode wheels in the embodiment of my invention described above may be varied within wide limits and the optimum rate of rotation will depend upon the 20 electrical current density, the nature of the electrolyte, operating temperature, the nature of the liquid metal electrode and the amount of alkali metal in the liquid metal electrode. The only limiting factor in regard to the speed of rotation 25 is that of centrifugal force. That is, the wheels should not be operated at such excessive speed that the liquid film on the upper portion thereon tends to be thrown off the wheel by centrifugal force developed by the rotation. For this reason, 30 the maximum possible speed of rotation may vary, depending upon the diameter of the wheel and also on the viscosity of the liquid metal film, which viscosity will vary depending upon the 35 amount of alkali metal dissolved in the liquid metal film, the nature of the liquid metal and also to some extent upon the temperature of operation. I have found, for example, that a steel 40 wheel three inches in diameter may be operated at a speed of up to about 100 revolutions per minute with little or no tendency for the liquid film to be thrown off, even with very low amounts of alkali metal in the film, the liquid metal being mercury. In general I prefer to operate at 45 much lower speeds, for example, for a three inch 50 steel wheel, using liquid mercury as electrode, I 55 prefer to rotate the wheel at about 15 to 25 revolutions per minute.

It will be obvious from the above description 60 that numerous modifications of my herein described invention may be made without departing from the spirit and scope thereof. The principle 65 of my invention is to provide a composite electrode which consists of a solid surface coated with an adherent film of liquid metal and means for contacting the solid surface first with a reservoir of liquid metal and then with an electrolyte, whereby a substantially continuous film of liquid metal adhering to the solid surface serves as active 70 electrode surface. My invention also includes the application of this principle to a double-cell electrolytic process with a liquid metal exchange electrode for electrolyzing (1) an aqueous solution with the liquid metal as cathode and (2) a 75 low-melting fused electrolyte with the liquid metal

as anode. In the modification described above by way of illustrating my invention a rotating wheel or disc is utilized for this purpose, the rotation of the wheel serving to coat the solid surface with liquid metal, contact it with the electrolyte and then again bring it into contact with the reservoir of molten metal whereby the metal film, after it has momentarily served as electrode is wholly or partially replaced by fresh liquid metal. In place of a rotating wheel for this purpose I may utilize a continuously moving band or belt of sheet metal, one portion of which lies in a reservoir of liquid metal while another portion thereof lies in the electrolyte. In this modification, if desired, the electrolyte may be spaced directly above the reservoir of molten metal into which the lower portion of the band is immersed or if desired the electrolyte may be in a container placed off to one side of the liquid metal reservoir and on the same level therewith or above it or below it. Still another modification to be used in place of the rotating wheel in accordance with my invention comprises providing a solid surface of any desired shape which, by either rotary or reciprocal motion may be alternately dipped into a liquid metal reservoir and brought into contact with the electrolyte. This may be accomplished for example by suspending a sheet of steel from a crank shaft whereby on rotation of the crank, the sheet is alternately raised and lowered so that at first it is dipped into a molten metal reservoir and then may be raised into the super-natant electrolyte. The same effect is also accomplished by providing a wheel of radiating spokes in place of the solid-faced wheel described above and shown in the appended drawings.

In still another modification of my invention, I may pass a solid metal surface through liquid metal to pick up an adherent film, contact the film-coated surface with the electrolyte to serve as electrode, whereby alkali metal is liberated and alloyed with the film and finally move the surface with adhering alloy film into contact with a substance reactive with alkali metal (e. g.; water) or utilize the alloy film-covered surface directly as anode in a "hot cell." Thus, an endless band of flexible steel or equivalent means may be used to carry a film of mercury or alkali metal amalgam coated thereon through a "cold cell" as cathode, thence back to the "cold cell." At a suitable point, the band may be passed through a reservoir of mercury to replenish the little lost by evaporation in the "hot cell." By this means, the power required to circulate mercury and the total amount of mercury required is still further diminished.

Various other means of alternately coating metal surfaces and bringing them into contact with electrolyte will be obvious to the skilled mechanician. I prefer, however, to use the herein described rotating disc for this purpose, since in this manner efficient transfer of a film of molten metal from molten metal reservoir to electrolyte may be obtained with the least complexity of moving parts, the simplest type of cell design and greatest overall efficiency. Also I have found that the greatest cell efficiency is obtained when the rotating wheel is in the form of a relatively thin disc, so arranged that at least the major portion of both of the plane sides of the disc dip into the mercury or amalgam in the manner shown in the appended drawings. This arrangement provides a larger active surface, as compared with a rotating cylinder, where only one side of the

cylindrical surface is utilized. Also, in my preferred modification, using the rotating discs, the amalgamated surface acting electrode forms an extended vertical electrode surface; this is the best arrangement, since it brings the electrode surface into contact with electrolyte substantially throughout the electrolyte and permits electrolysis products, e. g. gases or molten light metals, to readily and quickly pass upwardly out of the zone of electrolysis.

The utilization of my above described liquid metal film is not confined to electrolytic processes. Thus, it may advantageously be used to contact an alkali metal amalgam with a substance reactive with the alkali metal, to produce alkali metal compounds, e. g., hydroxides. For example sodium hydroxide may be produced by circulating sodium amalgam through an apparatus having a reservoir for the amalgam and rotating discs or their equivalent dipping into the amalgam in the reservoir, the upper portions of the rotating discs being in contact with a body of water or dilute sodium hydroxide solution which may be circulated or replenished as desired. In a similar manner a liquid alkali metal alloy may be brought into contact with a gaseous substance reactive with the alkali metal.

My herein described method and apparatus is especially well adapted for the production of alkali metal hydroxides by reacting amalgam with water. In a preferred form of my invention for this purpose, I may employ an electrolytic cell similar to the "cold cell" shown in Figs. 1 and 2 to produce the alkali metal amalgam. For reacting the amalgam with water, I may employ a decomposition cell similar to either of the cells shown by the drawings or a cell of simpler design, which preferably is constructed of iron or steel. Such decomposition cell would be similar to the cells of the drawings, having one or more rotating steel discs, the lower half of which dip into a well or wells of the amalgam, and the upper portion extending into water or dilute caustic solution. Preferably, graphite electrodes, similar to the cathodes 30 of Figs. 1 and 3, are arranged in close juxtaposition to the portions of the discs in the aqueous medium. These graphite electrodes are electrically connected with the amalgam in the well or wells, for example by being joined to the walls of the cell, which may be made of steel. The amalgam is circulated between the two cells in the manner illustrated by Fig. 1, except that the heat exchanger 18 may be eliminated. Water is circulated through the upper portion of the decomposition cell, and the resulting caustic solution leaving the cell may be evaporated to recover the solid alkali metal hydroxide. Since the decomposition cell may be operated at ordinary temperatures (e. g. 15 to 30° C.) the cell need not be insulated. Hydrogen evolved by the reaction may be allowed to escape into the air or may be collected by means of a suitable collecting dome, e. g. one similar to dome 33 of Figs. 1 and 3. By means of this arrangement and method caustic soda or other caustic alkali may be produced in good yield and with excellent power efficiency.

Also, my invention is not restricted to utilizations employing mercury as a carrier for alkali metals, but is also applicable to the use of other liquid metal electrodes, e. g. molten lead, lead alloys, alloys of bismuth, tin, lead and cadmium, such as "Woods metal" and the like.

A further advantage and utilization of the herein described invention resides in the

tion of the moving surfaces coated with adherent liquid metal film as a heat exchange device. For example, in the use of the rotating disc composite cathode described above for electrolysis of 5 a salt solution, the amalgam-coated rotating disc effectively acts as a heat exchange means to extract heat from the solution undergoing electrolysis. This results in increased electrolysis efficiency and also makes possible accurate control 10 of the temperature of the electrolyte when this is desired. I have found that in such operations, the temperature of the electrolyte is at all times during periods of extended operation maintained substantially identical with that of the 15 amalgam into which the rotating discs are immersed.

As a further example of such heat exchange action, the use of the moving amalgam-coated surfaces described herein for reacting alkali metal amalgams with gases or liquids reactive with the alkali metal may be mentioned. In such operations ordinarily there is more or less heat evolved by the reaction, and by means of the apparatus and method described herein the reaction 20 heat is effectively removed, especially in the case of reaction with liquids such as water, with the result that the reacting liquid is at all times maintained at substantially the same temperature as that of the underlying mass of amalgam. 25 In the case of endothermic reactions, by supplying heat to the underlying reservoir of liquid metal or amalgam, heat is effectively supplied to the reacting liquid by the heat exchange effect above described. In either case, the reaction 30 temperature may be controlled within narrow 35 limits by this means.

My invention is also applicable to heat exchange operations in the absence of electrolysis or other chemical action. For example, a liquid 40 may be effectively cooled by use of the herein described rotating bodies having an adherent liquid metal coating, which bodies are partially immersed in a reservoir of the metal and extend into the liquid to be cooled. By supplying heat to 45 or extracting heat from the underlying reservoir of liquid metal, the temperature of the liquid to

be cooled or heated thus may be controlled within very narrow limits. If desired, liquid alkali metal amalgams containing sufficient alkali metal to cause the amalgam to adhere to the metallic surface may be utilized in such heat exchange 5 operations. Such adaptations may be used for example to cool liquids which are not reactive with alkali metals (e. g. hydrocarbons) when it is desired to carry on the heat exchange operation without chemical reaction or without destruction 10 of the alkali metal utilized. This heat exchange method and apparatus also may be used to add or subtract heat from reactions in which there are no reactants or products which are reactive with the alkali metal amalgam. 15

I claim:

1. An electrolytic cell comprising a container, having electrically conductive interior side walls, a body of liquid metal adapted to serve as an electrode in the lower portion of said container, an electrolyte floating on the surface of said liquid metal and a metal shield within said container and spaced from the side walls thereof extending through said electrolyte close to but out of contact with said liquid metal and electrically insulated from said side walls. 25

2. An electrolytic cell comprising a container having interior side walls of metal, a liquid metal anode in the lower portion of said container, an electrolyte floating on the surface of said liquid 30 metal anode, and a metal shield close to but electrically insulated from said side walls, which shield extends through said electrolyte close to but out of contact with said anode.

3. An electrolytic cell comprising a container 35 having interior side walls of metal, a liquid metal anode in the lower portion of said container, an electrolyte floating on the surface of said liquid metal anode, and a metal shield close to but electrically insulated from said side walls, which 40 shield extends through said electrolyte close to but out of contact with said anode and at least one rotatable disc so positioned in the cell with substantially horizontal axis that it lies partly in said electrolyte and partly in said liquid anode. 45

HARVEY N. GILBERT.